

## 1

3,031,410

## COMPOSITION AND METHOD OF INHIBITING CORROSION OF FERROUS METALS BY AMINE-STABILIZED UNSATURATED CHLORINATED HYDROCARBONS

Wilbur H. Petering and William A. Callahan, Detroit, Mich., assignors to Detrex Chemical Industries, Inc., Detroit, Mich., a corporation of Michigan  
No Drawing. Filed June 10, 1958, Ser. No. 741,001  
14 Claims. (Cl. 252—171)

This application is a continuation-in-part of applicants' copending application Serial No. 445,474, filed July 23, 1954, and now abandoned.

This invention relates to a composition and method of inhibiting the corrosion of ferrous metals by amine-stabilized, unsaturated chlorinated hydrocarbons, particularly those chlorinated hydrocarbons which decompose under the influence of metals or oxygen to form acidic products. Among the chlorinated hydrocarbons inhibited in accordance with this invention are the unsaturated chlorinated hydrocarbons such as 1,2 dichloroethylene, trichlorethylene, perchlorethylene, the chloropropylanes, the chlorobutylanes and the chlorobutadienes. All such unsaturated chlorinated hydrocarbons have low molecular weights and are subject to decomposition by metals or oxygen, or in their presence, and this decomposition is accelerated by light and heat.

It is conventional in the art to add stabilizers of various types to chlorinated hydrocarbons. Among the accepted stabilizers are the phenolic compounds, aryl amines, and various azo compounds. However, the use of such compounds is quite limited except in the case of a few of the higher boiling chlorinated hydrocarbons, since the stabilizers also have relatively high boiling points. A wide difference in boiling points between the solvent and the stabilizer is undesirable because of the difficulty of stabilizing the vapor phase, and it is desirable to provide a combination of solvent and stabilizer not having a wide difference in boiling points.

The organic amine bases have enjoyed widespread use as stabilizers for unsaturated chlorinated hydrocarbons. Such bases, including primary aliphatic amines having the NH<sub>2</sub> radical and basic cyclic compounds characterized by nitrogen in the ring such as pyridine and the like are disclosed in the patents to Dinley, Numbers 2,096,735, 2,096,736 and 2,096,737. Under many conditions the primary aliphatic and cyclic amine bases disclosed in the Dinley patents are highly effective and desirable stabilizers for chlorinated hydrocarbons.

In the manufacture of the unsaturated chlorinated hydrocarbons as trichlorethylene, for example, the recovery of a neutral, sweet, relatively pure product is almost impossible without the use of a stabilizer such as these amines. The amine stabilizer should be present in the refining operation, as distinguished from adding amine to the refined product, and the amine should be volatile with the chlorinated hydrocarbon and therefore carry over from the refining operation into the refined product. Unless a neutral, sweet product is obtained when the solvent is refined, subsequent attempts to stabilize the solvent often prove futile, or at least extremely costly and time consuming. Thus, the amines are not only highly effective and desirable stabilizers, but their use in both the liquid and vapor in the last stages of manufacture is almost essential.

Yet, in spite of the effectiveness and desirability of the amines as stabilizers, there appears to have been an undesirable reaction or set of reactions which take place when the amines are used as stabilizers in unsaturated chlorinated hydrocarbon solvents in the presence of certain metals of the iron group. It has now been discovered that the lower boiling unsaturated chlorinated hydrocar-

## 2

bons, when stabilized with certain of the conventional organic amines, such amines having boiling points which are not widely different from the boiling point of the chlorinated hydrocarbon, appear to enter into a complex reaction when exposed to one of those metals. The reaction appears to be metal-induced, causing a progressive decomposition of the chlorinated hydrocarbons. The reaction which occurs in the presence of conventional amines causes attack on the metal, rapid loss of amine stabilizer and the development of acidic materials, and apparently the series of reactions producing the decomposition requires the presence of the amine.

The corrosive action of the amines appears to be related to certain specific metals, especially iron (also in its common alloyed form as steel) and copper (alone or in its alloyed form as brass). On the other hand, aluminum, which is known to be an agent for metal induced decomposition in some cases, does not initiate the corrosion reaction in amine-stabilized systems.

In referring to "amines" in the foregoing paragraph, we have used the term in its broad sense. The other organic bases specified in the Dinley patents, including cyclic compounds characterized by nitrogen in the ring, such as pyridine and morpholine, for example, are included within the meaning of this term. Among the suitable amines which are listed in the examples set forth hereinafter, and which are accordingly suitable in the practice of this invention are pyridine, disec butylamine, diisopropylamine, diethylamine, n-butylamine, amylamine, methyl pyridine, n-methyl morpholine, triethylamine, and hexylamine.

The exact mechanism by which the amine reacts with the chlorinated hydrocarbon in the presence of the metal is not completely known or understood. It may be that the amine, being a strong base, that is, a Lewis base and an electron donor, either forms a covalent bond with one carbon atom of the unsaturated chlorinated hydrocarbon, and the resulting fragment reacts with the metal, or, in the case of chlorinated hydrocarbons containing hydrogen, the amine may react by first removing a hydrogen to yield "ionic" fragments which in turn are reactive toward metals—the end products of such reactions being more or less complex metal-organic chloro compounds. Then again, the metal may be the initiator of the set of reactions which involve the amine and the chlorinated solvent.

One explanation for the reaction is that the unsaturated chlorinated compound, being amphoteric, that is, having one carbon basic and the other acid at the unsaturated bond, and the amine being basic, that is, a Lewis base and an electron donor, forms a covalent bond at the acidic carbon leaving the resultant fragment basic and that a metal brings about chelation. It may be that the basic fragment, or the electron donor amine itself holds the metal in the active state as opposed to the passive state (according to the Electron Theory of Corrosion in Corrosion Handbook by Uhlig) so that the active metal reacts with the solvent or the amine stabilizer, forming organo-metallics which are agents which hasten normal oxidation or at least remove the stabilizer as such and thus reduce the concentration of stabilizer to sub minimal levels, and at the same time cause serious attack on or corrosion of the metal. In any event, serious corrosion problems are encountered when a low-boiling unsaturated chlorinated hydrocarbon is stabilized with an amine and the product exposed to a ferrous metal, or copper, particularly when the hydrocarbon is a hot, bone-dry liquid.

It is accordingly an object of this invention to provide a composition and method for overcoming the foregoing disadvantages. Still another object is to provide an improved corrosion-resistant stabilizer composition

for the lower boiling unsaturated chlorinated hydrocarbons. Other objects and advantages of this invention will further appear hereinafter.

In accordance with this invention, the corrosive action of the organic amine in the presence of metals in the chlorinated hydrocarbon is overcome by incorporating into the mixture a small amount of a substituted aliphatic epoxy compound which interferes with the corrosive action of the amine in the presence of ferrous metals. The substituted aliphatic epoxy compound does not interfere with the stabilizing action of the amine or its ability to act as an alkaline material or to act as a reducing agent. It appears that these substituted aliphatic epoxy compounds act to retard or interfere with the corrosive activity of the amine by either hindering the amine itself, or by forming a protective layer over the surface of the metal. In the former case the amount of substituted aliphatic epoxy compound required to control the action of the amine is related to the amount of amine used, while in the latter case the amount of substituted aliphatic epoxy compound required is related to the surface area of the metal exposed to the solvent and amine.

It has been found that in a few cases, if the amine, when used in the usual stabilizing concentration, reacts with the chlorinated solvent and the metal exposed to the stabilizer and solvent, the activity can be reduced by using a greatly increased concentration of stabilizer as, for example, about ten times the usual stabilizing amount. It is believed that the very large amount of amine stabilizer is able to form a protective coating over the metal surface, thus interfering in the reaction between the amine, solvent and metal. That method of controlling the activity of amine is not desirable because such large amounts of amine add to the cost of stabilizing the solvent; moreover, if under some condition the concentration of amine should become depleted, the concentration would fall into that level where the reactivity of the amine would rapidly increase and the corrosion difficulties mentioned above would be encountered.

The substituted aliphatic epoxy compounds of this invention have the following general formula:



Where R may be an alkyl radical such as  $\text{C}_x\text{H}_{2x+1}$ , where x is an integer from 1 to 3, or an alkene group or a prenyl group, the following substituted aliphatic epoxy compounds are illustrative:

(1) Glycidyl methyl ether



(2) Glycidyl ethyl ether



(3) Glycidyl isopropyl ether



(4) Glycidyl phenyl ether



(5) Glycidyl allyl ether



In accordance with this invention, the crude unsaturated chlorinated hydrocarbon, prior to the refining operation, is combined with an inhibitive proportion of amine. The stabilized product is combined with an inhibitive proportion of a substituted aliphatic epoxy compound as described above.

In accordance with this invention, the crude unsaturated chlorinated hydrocarbon, prior to the refining operation, is combined with a stabilizing proportion of amine. The stabilized product is combined with an inhibitive proportion of a substituted aliphatic epoxy compound as described above. The resulting mixture is heated in a still, which volatilizes the amine and chlorinated hydrocarbon. The substituted aliphatic epoxy compound may be only partially volatilized. Since the severe corrosion problem occurs in the substantially anhydrous liquid phase, the substituted aliphatic epoxy compound is retained at the location where it is most needed. At the same time, the amine stabilizes the chlorinated hydrocarbon in the liquid and vapor phases.

Unsaturated chlorinated hydrocarbons such as trichloroethylene and perchloroethylene are widely used as degreasers, cleaners and the like. For example, ferrous metals are degreased commercially by subjecting them to liquid and to vapor phase chlorinated hydrocarbons. Since the liquid hydrocarbon is heated and contains amine, and since it is anhydrous and in the liquid phase, there is some danger of corrosion of the degreasing apparatus or of the metal immersed in the liquid. Accordingly, it is commercially advantageous to provide a chlorinated hydrocarbon solvent which contains both an amine and a substituted aliphatic epoxy compound in accordance with this invention.

It is well known that the proportions of amine stabilizers may vary from trace values (such as .01% by weight or less) to as high as 1.0% by weight, based on the weight of the chlorinated hydrocarbon. However,

35 a range of the order of about .02-.20% by weight represents the proportions considered commercially preferable in most amine-stabilized chlorinated hydrocarbons. Amine stabilizers have been well known and extensively used, and different amines have been used in different proportions for different chlorinated hydrocarbons. The art is well aware of the proper proportions of each specific amine stabilizer in each specific chlorinated hydrocarbon, and such proportions are conventionally referred to as "stabilizing proportions," and are so defined herein.

40 45 The proportions of the substituted aliphatic epoxy compound may be varied from about .01% by weight to about 5% by weight, but a range of about .01-.15% by weight is preferred. Such proportions are referred to as "inhibitive proportions," and are so defined herein. Preferably, the weight of substituted aliphatic epoxy compound is about 1-5 times the weight of amine stabilizer. The effect of these substituted aliphatic epoxy compounds is shown in the results of tests described below:

45 50 A chlorinated hydrocarbon is refluxed in the presence of a weighed piece of metal. A stabilizing amount of an amine is added and the solvent refluxed continuously. After refluxing for at least 48 hours the solvent is titrated for alkalinity and the metal weighed to determine the loss of metal. Similar tests, in which an inhibiting amount of substituted aliphatic epoxy compound has been added along with the amine, are run. Also tests, in which the substituted aliphatic epoxy compound is used alone without amine, are run.

55 60 As used throughout the present specification and claims, the term "substituted aliphatic epoxy compound" is intended to define the type compounds referred to in the specification hereof, in which all of the substituent groups comprise carbon and hydrogen with oxygen appearing as indicated in the general formula. Epoxy compounds containing halogen are thus specifically excluded from the substituted aliphatic epoxy compounds of the present invention.

65 70 The foregoing reflux test has been used in industry to evaluate chlorinated solvents for use in such processes as degreasing. Since the test is not particularly severe it

does not evaluate stability of the solvent or the efficacy of the stabilizer used. Therefore in the absence of a stabilizer or in the presence of a weak stabilizer, the breakdown of the solvent is not particularly rapid. Therefore, because the test duplicates a continuous refluxing condition which would exist under normal conditions of use, it serves as a valuable tool in showing the reaction of the amine and solvent in the presence of metal.

and hexylamine, and having a boiling point near that of the chlorinated hydrocarbon in a stabilizing proportion in an amount of from about .01% to about 1.0% by weight of said solvent, said amine-stabilized solvent in the presence of ferrous metals causing metal corrosion, in combination with an inhibitor for said ferrous-metal amine corrosion comprising a glycidyl ether corresponding to the general formula

TABLE IA  
*Inhibitory Effect on Steel of Substituted Epoxy Compounds in Trichlorethylene*

| Amine                            | Amine,<br>percent<br>by weight | Subst. Epoxy Compound Added,<br>percent by weight | Hours<br>of Test | Loss of<br>Alkalinity,<br>p.p.m. HCl | Loss of Metal,<br>Mgm./Ft. <sup>2</sup> |
|----------------------------------|--------------------------------|---------------------------------------------------|------------------|--------------------------------------|-----------------------------------------|
| Triethylamine (Commercial Grade) | .02                            | None-----                                         | 39.5             | 82.0                                 | 3,800.                                  |
| Do-----                          | .02                            | .08% Glycidyl Methyl Ether-----                   | 116.0            | 50.0                                 | No Corrosion.                           |
| Do-----                          | .02                            | .10% Glycidyl Methyl Ether-----                   | 116.0            | 43.2                                 | Do.                                     |

TABLE IB  
*Inhibitory Effect on Steel of Substituted Epoxy Compounds in Perchlorethylene*

| Amine                       | Percent | Subst. Epoxy Compound Added, percent | Hours of Test | Loss of Alkalinity, p.p.m. HCl | Loss of Metal, Mgm./Ft. <sup>2</sup> |
|-----------------------------|---------|--------------------------------------|---------------|--------------------------------|--------------------------------------|
| Pyridine (Commercial Grade) | .02     | None                                 | 120           | 59.4                           | 122.                                 |
| Do                          | .20     | do                                   | 120           | 230.0                          | 348.                                 |
| Do                          | .02     | .05% Glycidyl methyl ether           | 72            | 65.0                           | No Corrosion.                        |
| Do                          | .02     | do                                   | 88            | 64.0                           | Do.                                  |
| Do                          | .02     | .02% Glycidyl methyl ether           | 88            | 65.0                           | Do.                                  |
| Do                          | .02     | .01% Glycidyl methyl ether           | 88            | 75.0                           | Do.                                  |
| Do                          | .02     | .005% Glycidyl methyl ether          | 88            | 75.0                           | Corrosion.                           |
| Do                          | .02     | .002% Glycidyl methyl ether          | 88            | 75.0                           | Do.                                  |
| Me-Morpholine               | .02     | None                                 | 72            | 72.0                           | 585.                                 |
| Do                          | .10     | do                                   | 72            | 96.3                           | 668.                                 |
| Do                          | .02     | .05% Glycidyl methyl ether           | 87            | 56.7                           | No Corrosion.                        |
| Do                          | .02     | .05% Glycidyl isopropyl ether        | 87            | 61.0                           | Do.                                  |
| Do                          | .02     | .05% Glycidyl allyl ether            | 87            | 59.0                           | Do.                                  |
| Triethylamine               | .02     | None                                 | 16            | 71.0                           | Heavy Corrosion.                     |
| Do                          | .02     | .05% Glycidyl methyl ether           | 96            | 46.0                           | No Corrosion.                        |
| Do                          | .02     | do                                   | 88            | 46.0                           | Do.                                  |
| Do                          | .02     | .02% Glycidyl methyl ether           | 88            | 72.0                           | Do.                                  |
| Do                          | .02     | .01% Glycidyl methyl ether           | 88            | 74.2                           | Do.                                  |
| Do                          | .02     | .005% Glycidyl methyl ether          | 88            | 75.4                           | Corrosion.                           |
| Do                          | .02     | .002% Glycidyl methyl ether          | 88            | 75.4                           | Do.                                  |
| Do                          | .02     | .05% Glycidyl methyl ether           | 144           | 51.0                           | No Corrosion.                        |
| Do                          | .02     | .10% Glycidyl methyl ether           | 144           | 41.6                           | Do.                                  |
| Do                          | .02     | .05% Glycidyl methyl ether           | 87            | 41.0                           | Do.                                  |
| Do                          | .02     | .05% Glycidyl isopropyl ether        | 87            | 55.5                           | Do.                                  |
| Do                          | .02     | .05% Glycidyl allyl ether            | 87            | 38.7                           | Do.                                  |

The beneficial effects observed in Tables IA and IB 50 were not the result of a stabilizing property of the substituted epoxy compound itself. Several anti-oxidants or stabilizers which are known in the art and accepted as effective inhibitors were added to the chlorinated solvent along with an amine. No inhibitory effects on the action of the amine were observed. If anything, the activity of the amine was increased, as indicated by the fact that attack on the metal was initiated somewhat sooner than when the amine is present alone. Also, in a number of cases, the tests were discontinued while the solvent was still alkaline, and in spite of this fact, considerable attack on the metal had already taken place. This indicates that the corrosive action on the metal is not the result of a lack of stabilizer or the action of an unstable solvent. 55 60

Having thus described our invention, we claim:

1. A stabilized solvent which is substantially non-corrosive to ferrous metals consisting essentially of a volatile low-boiling low molecular weight unsaturated chlorinated hydrocarbon selected from the group consisting of trichlorethylene and perchlorethylene, and which is normally subject to decomposition by metals and oxygen containing an organic amine selected from the group consisting of pyridine, di-sec. butylamine, diisopropylamine, diethylamine, n-butylamine, amylamine, methyl pyridine, N-methyl morpholine, triethylamine,



55 where R is selected from the group consisting of an alkyl radical having the formula  $C_xH_{2x+1}$ , where x is an integer from 1 to 3, the allyl radical and the phenyl radical, said corrosion inhibitor being present in an amount from about .01%--5% by weight.

2. The stabilized solvent defined in claim 1 wherein  
60 the glycidyl ether is glycidyl methyl ether.

3. The stabilized solvent defined in claim 1 wherein  
the glycidyl ether is glycidyl ethyl ether.

4. The stabilized solvent defined in claim 1 wherein  
the glycidyl ether is glycidyl isopropyl ether.

65 5. The stabilized solvent defined in claim 1 wherein  
the glycidyl ether is glycidyl phenyl ether.

6. The stabilized solvent defined in claim 1 wherein  
the glycidyl ether is glycidyl allyl ether.

70 7. In a process wherein a volatile unsaturated low  
molecular weight chlorinated hydrocarbon selected from  
the group consisting of trichlorethylene and perchlor-  
ethylene, is exposed in the hot anhydrous liquid state to  
a ferrous metal, said hydrocarbon including a stabilizing  
proportion of an organic amine selected from the group  
75 consisting of pyridine, di-sec. butylamine, diisopropyl-

7  
amine, diethylamine, n-butylamine, amylamine, methyl pyridine, N-methyl morpholine, triethylamine and hexylamine, and which normally reacts with the chlorinated hydrocarbon and ferrous metal in the presence of said metal to corrode said metal, the amount of said amine being from about .01% to about 1.0% by weight of said solvent, the improvement which comprises incorporating into the said chlorinated hydrocarbon and amine about .01-5% by weight of an inhibitor for said ferrous metal-amine corrosion comprising a glycidyl ether having the general formula



where R is selected from the group consisting of an alkyl radical having the formula  $C_xH_{2x+1}$ , where x is an integer from 1 to 3, the allyl radical and the phenyl radical.

8. The process defined in claim 7 wherein the glycidyl ether is glycidyl methyl ether.

9. The process defined in claim 7 wherein the glycidyl ether is glycidyl ethyl ether.

10. The process defined in claim 7 wherein the glycidyl ether is glycidyl isopropyl ether.

11. The process defined in claim 7 wherein the glycidyl ether is glycidyl phenyl ether.

12. The process defined in claim 7 wherein the glycidyl ether is glycidyl allyl ether.

13. A stabilized solvent which is substantially non-corrosive to ferrous metals consisting essentially of a volatile low-boiling low molecular weight unsaturated chlorinated hydrocarbon selected from the group consisting of trichlorethylene and perchlorethylene, which is normally subject to decomposition by metals and oxygen, containing as a stabilizer about .01%-20% of an organic amine selected from the group consisting of pyridine, di-sec. butylamine, diisopropylamine, diethylamine, n-butylamine, amylamine, methyl pyridine, N-methyl morpholine, triethylamine, and hexylamine, and having a boiling point near that of the chlorinated hydrocarbon, said amine-stabilized solvent in the presence of

5  
10  
15  
20  
25  
30  
35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985  
7990  
7995  
8000  
8005  
8010  
8015  
8020  
8025  
8030  
8035  
8040  
8045  
8050  
8055  
8060  
8065  
8070  
8075  
8080  
8085  
8090  
8095  
8100  
8105  
8110  
8115  
8120  
8125  
8130  
8135  
8140  
8145  
8150  
8155  
8160  
8165  
8170  
8175  
8180  
8185  
8190  
8195  
8200  
8205  
8210  
8215  
8220  
8225  
8230  
8235  
8240  
8245  
8250  
8255  
8260  
8265  
8270  
8275  
8280  
8285  
8290  
8295  
8300  
8305  
8310  
8315  
8320  
8325  
8330  
8335  
8340  
8345  
8350  
8355  
8360  
8365  
8370  
8375  
8380  
8385  
8390  
8395  
8400  
8405  
8410  
8415  
8420  
8425  
8430  
8435  
8440  
8445  
8450  
8455  
8460  
8465  
8470  
8475  
8480  
8485  
8490  
8495  
8500  
8505  
8510  
8515  
8520  
8525  
8530  
8535  
8540  
8545  
8550  
8555  
8560  
8565  
8570  
8575  
8580  
8585  
8590  
8595  
8600  
8605  
8610  
8615  
8620  
8625  
8630  
8635  
8640  
8645  
8650  
8655  
8660  
8665  
8670  
8675  
8680  
8685  
8690  
8695  
8700  
8705  
8710  
8715  
8720  
8725  
8730  
8735  
8740  
8745  
8750  
8755  
8760  
8765  
8770  
8775  
8780  
8785  
8790  
8795  
8800  
8805  
8810  
8815  
8820  
8825  
8830  
8835  
8840  
8845  
8850  
8855  
8860  
886

UNITED STATES PATENT OFFICE  
CERTIFICATE OF CORRECTION

Patent No. 3,031,410

April 24, 1962

Wilbur H. Petering et al.

It is hereby certified that error appears in the above numbered patent requiring correction and that the said Letters Patent should read as corrected below.

Column 4, lines 1 to 3, strike out "In accordance with this invention, the crude unsaturated chlorinated hydrocarbon, prior to the refining opamine. The stabilized product is combined with an n-"; column 5, line 64, for "ustable" read -- unstable --.

Signed and sealed this 9th day of October 1962.

(SEAL)

Attest:

ERNEST W. SWIDER  
Attesting Officer

DAVID L. LADD  
Commissioner of Patents